# EUROPEAN PATENT APPLICATION

(11) **EP 1 449 936 A1**
(43) Date of publication of application: **25.08.2004**
(21) Application number: 02779915.4
(22) Date of filing: 16.10.2002
(51) Int. Cl.: C23C 22/07, C23C 22/40, C10M 173/00

(54) **PROCESS FOR PRODUCING METAL WIRE ROD FOR PLASTIC WORKING**

(30) Priority: 19.10.2001 JP 2001322574
(71) Applicant: NIHON PARKERIZING CO., LTD., Chuo-ku, Tokyo 103-0027 (JP)
(72) Inventor: YOSHIDA, Masayuki, c/o Nihon Parkerizing Co., Ltd., Tokyo 103-0027 (JP); KOMIYAMA, Shinobu, c/o Nihon Parkerizing Co., Ltd., Tokyo 103-0027 (JP); TSUIKI, Yugo, c/o Nihon Parkerizing Co., Ltd., Tokyo 103-0027 (JP)
(74) Representative: Endres, Helmut
(86) International application number: PCT/JP2002/010750
(87) International publication number: WO 2003/035929

(57) **Abstract**

A method for preparation of the metal wire rod for plastic processing comprising, carrying out cleaning treatment by at least one kind of cleaning treatment method selected from the group consisting of shot blast, sand blast, bending and acid cleaning of cathode and anode on the surface of metal wire rod of 0.3-50 mm diameter for 20 seconds or less, contacting with aqueous lubricious film formation treating solution which contains at least one kind of inorganic salt selected from the group consisting of phosphate, sulfate, borate, silicate, molybdate or tungstate and at least one kind of slipping agent selected from the group consisting of metal soap, wax, polytetrafluoroethylene, molybdenum disulfate and graphite, wherein, the weight ratio of solid of said slipping agent/inorganic salt is within the limit from 0.1 to 4.0 for 5 seconds or less, drying immediately and forming lubricious film of adhesion amount from 0.5 to 20 g/m² on the surface of the wire rod by continuous inline system. The method allows the preparation of a metal material for plastic processing having excellent lubricating characteristics in a short time.

## Description

### FIELD OF THE INVENTION

The present invention relates to a method for inline preparation of metal wire rod used for plastic processing which provides excellent lubricity to the surface of metal wire rod such as steel, stainless steel, titanium or aluminum without carrying out chemical conversion treatment. More in detail, the present invention relates to the method for inline preparation of film having excellent lubricity on the surface of metal wire rod such as steel, stainless steel, titanium or aluminum without carrying out chemical conversion treatment when the cold plastic processing such as header processing is carried out.

### DESCRIPTION OF THE PRIOR ART

In general, in the case when the metal material such as steel or stainless steel is plastically processed, lubricious film is generated on the surface of metal aiming to prevent from burning and sticking or scoring caused by the metal contact between a material to be processed and a tool. As a kind of above mentioned lubricious film, a type which makes lubricant physically stick on the surface of metal or a type which use lubricant after generation of chemical conversion treatment film on the surface of metal. The type which makes lubricant physically stick on the surface of metal is inferior in adhesion to the type which uses lubricant after generation of chemical conversion treatment film on the surface of metal, therefore generally this type is used for the light processing. In the case which uses lubricant after generation of chemical conversion treatment film on the surface of metal, it is ordinary to use a lubricant having slippery characteristics after generation of a phosphate film or an oxalate film which acts the role of a carrier on the surface. This type is characterized to have a structural feature of double layers consisting of a chemical conversion treatment film as a carrier film and a lubricant, and shows very high resistance to burning and sticking. Therefore, this type has been widely used in the plastic processing field such as wire drawing, tube drawing or forging. Especially in the most serious processing among the plastic processings, the method to form an undercoating film such as phosphate film or oxalate film on the surface of metal and to use lubricant on said film is frequently used.

Further, the lubricants used on chemical conversion treatment film can be divided to two groups according to the method for use. One is the group to stick lubricant physically to the chemical conversion treatment film, another one is the group to stick lubricant to the chemical conversion treatment film by means of chemical reaction. As the lubricants belonging to the former group, a lubricant using mineral oil, vegetable oil and synthetic oil as the base oil and to which an extreme-pressure additive is added or a lubricant prepared by dispersing solid lubricant such as graphite or molybdenum disulfide in water with binder component, which is used in the sticking or the drying process, can be mentioned. Since these lubricant can be simply used by spray coating or by dipping coating, have a merit that the preservation management of liquid is not necessary, however, because of the lubricity, is mainly used for light lubrication. On the contrary, the lubricants belonging to the latter group, the reaction type soap such as sodium stearate is used and is used only in the case that requires strong lubricity.

However, when the chemical conversion treatment accompanied with chemical reaction and the reaction type soap are used, high lubricity ca be obtained, on the contrary, the control of liquid, temperature adjusting to control the chemical reaction, the wasting and the renewal of liquid accompanied with the deterioration of liquid are becoming necessary. Aiming the recent environmental maintenance of the earth, the decreasing of the industrial waste is becoming a big theme. Accordingly, the lubricant or the treating method which does not cause the waste is desired. Further, because the process and the control of the treating liquid are complicated, the simple treating method is desired.

In the meanwhile, the lubrication treatment of metal wire rod is carried out on the strand of coil prepared by winding the metal wire rod by step by step. Namely, the lubrication treatment is carried out by batch processing. Generally, the strand of approximately 2 tons is dipped into a processing tank having 10 several ton volume and treated. Ordinary, after oil is removed by alkali degreasing and washing by water, dipped into a washing bath containing hydrochloric acid or sulfuric acid so as to remove scale. The temperature of this treatment is from ordinary temperature to 60°C and the time is several 10 minutes. Then washed by water, dipped into a chemical conversion bath and carry out the phosphate film treatment or oxalate film treatment. In the case of phosphate treatment, the treating temperature is approximately 80°C and treating time is approximately 10 minutes. After that, washed by water, dipped into soap treating bath and carry out the soap treatment. The treating temperature of this soap treatment is approximately 80°C and treating time is approximately 10 minutes. As mentioned above, the conventional method for treating is carried out by batch processing and several tanks of 10 several tons volume are necessary. Therefore, large space is needed for the treatment. Still more, since the treating temperature is high, the large energy is required for the temperature elevation and keeping the temperature. Furthermore, the treating time for each process is long, and about one hour is needed for the treatment of one strand.

Aiming to dissolve above mentioned problems, the lubricant composition whose base material is water soluble polymer or aqueous emulsion thereof and to which solid lubricant and chemical conversion film forming agent are blended (JP Laid open publication 52-20967) is proposed, however, the product being equal to the chemical conversion film treatment is not obtained. For the purpose to dissolve these mentioned problems, the inventors of the present invention, already proposed the aqueous lubricant for cold plastic processing on metal in which solid lubricant and oil are respectively dispersed and emulsifted homogeneously comprising, (A) water soluble inorganic salt, (B) solid lubricant and (C) at least one oil component selected from the group consisting of mineral oil, animal oil, vegetable oil and synthesized oil, (D) surfactant and (E) water (JP Laid open publication 10-8085). However, the lubricant by said invention, since the oil component is emulated, is not stable at the industrial use, and the excellent lubricity is not displayed stable.

Further, as the method to dissolve these problems, the inventors of the present invention also proposed the lubricant composition for plastic processing of metal comprising, (A) synthetic resin, (B) water soluble inorganic salt, wherein solid weight ratio (A)/(B) is from 0.25/1 to 9/1 and said synthetic resin is dissolved or dispersed (JP Laid open publication 2000-63880). However, the lubricant of this invention is mainly composed of synthetic resin and can not display stable the sufficient lubricity by serious processing condition. Further, in these references, there is a description about lubricity, however, the illustration about continuous inline treatment of metal wire rod is not complete.

The present invention is to dissolve the above mentioned problems, and the object of the present invention is to provide the method for preparation of metal wire rod for plastic processing which has excellent lubricity, concerning environmental maintenance of earth and can be processed in short time, by lower energy and in narrow space, further can be applied to various metal materials.

### DISCLOSURE OF THE INVENTION

The inventors of the present invention, carried out the intensive study to dissolve the above mentioned object and found out the novel method to prepare the metal wire rod whose surface is coated by lubricious film of specific amount by inline, by carrying out following processes continuously, that is, after specific cleaning treatment is carried out on the surface of said metal wire rod, the aqueous treating liquid containing specific component is contacted and coated then dried, thus the present invention is accomplished.

That is, the present invention is the method for preparation of the metal wire rod for plastic processing comprising, carrying out cleaning treatment by at least one kind of cleaning treatment method selected from the group consisting of shot blast, sand blast, bending and acid cleaning of cathode and anode on the surface of metal wire rod of 0.3-50 mm diameter for 20 seconds or less, contacting with aqueous lubricious film formation treating solution which contains at least one kind of inorganic salt selected from the group consisting of phosphate, sulfate, borate, silicate, molybdate or tungstate and at least one kind of slipping agent selected from the group consisting of metal soap, wax, polytetrafluoroethylene, molybdenum disulfate and graphite, wherein the weight ratio of solid of said slipping agent/inorganic salt is within the limit from 0.1 to 4.0, for 5 seconds or less, drying immediately and forming lubricious film of adhesion amount from 0.5 to 20 g/m² on the surface of the wire rod by continuous inline system.

In above mentioned method, the cleaning treated metal wire rod can be contacted with the aqueous lubricious film formation treating solution after previously heated by means of heating method such as high frequency heating, hot air heating, hot water heating, steam heating, direct heating or superheated steam heating.

As the above mentioned metal wire rod, the metal wire rod selected from the group consisting of iron, steel, stainless steel, aluminum, aluminum alloy, magnesium, magnesium alloy, titanium, titanium alloy, copper and copper alloy can be desirably used.

Further, it is desirable that the linear velocity of metal wire rod at the continuous treatment is from 10 to 150 m/minute.

By this method, it is possible to form the film having high lubricity on the metal wire rod by small energy, in small space, by simple method and in short time.

### BRIEF DESCRIPTION OF THE DRAWING

Fig.1 is the cross-sectional view of the bolt which is used at the test of header processability of the metal wire rod for plastic processing prepared by the method of the present invention.

### DESCRIPTION OF THE PREFFERED EMBODYMENT

The present invention will be illustrated in more detail with accordance to the following description. The term of cold plastic processing of the present invention mainly means the header processing. As the ordinary processing of this header processing, the preparation of a bolt can be mentioned. The wire rod is cut and process it as a bolt. Further, parts of car or machine are cut from wire rod and processed.

The metal material of the present invention is used for these cold processing, and the desirably to be one selected from the group consisting of iron, steel, stainless steel, aluminum, aluminum alloy, magnesium, magnesium alloy, titanium, titanium alloy, copper and copper alloy. In the present invention, the treatment of the metal wire rod is not carried out by the state of a coil shaped strand, that is, bundled shape (above mentioned batch system), but carried out by inline system which treat the metal wire rod continuously by individual state. The desirable diameter of the metal wire rod is in the limit from 0.3 to 50 mm. When the diameter is under 0.3 mm, the wire is too thin to form homogeneous coating by the present invention and causes a problem in the plastic processing. And when the diameter is thicker than 50 mm, there is no technical problem, but the unwinding or winding of the wire are very hard work, and is meaningless from the view point of the industrial use.

The cleaning treatment of the metal wire rod is necessary to be carried out by at least one kind of cleaning treatment method selected from the group consisting of shot blast, sand blast, bending and acid cleaning of cathode and anode. The term of cleaning treatment of the present invention means to remove the oxidation scale grown by annealing or various kind of stain (such as oil). By this cleaning treatment, the followed lubricious film formation can be carried out smoothly. Especially, in recent years, the reduction of the load to the wasted water treating equipment is desired from the view point of the environmental problem, and from this view point, the method so called mechanical de-scaling, by which no wasted water is discharged, that is, inline shot blast or bending are useful. Further, in the case which uses acid, the acid cleaning of cathode and anode using electrolysis is used for the purpose to shorten the treating time. The acid cleaning of anode uses acid such as sulfuric acid, uses wire rod as an anode and use counter electrode (platinum plate) as a cathode, and electrolyzes for several seconds by applied voltage 2-50V and current density 2-100 A/dm², so as to dissolve metal material partially and remove scale. While, the acid cleaning of cathode uses acid such as sulfuric acid, uses wire rod as a cathode and use counter electrode (platinum plate) as an anode, and electrolyzes for several seconds by applied voltage 2-50V and current density 2-100 A/dm², and remove scale by utilizing the effect of hydrogen gas which generates at the metal surface.

In the case of firm scale, it is effective to carry out the acid cleaning of anode then acid cleaning of cathode. Further, for the purpose to remove fine residue (such as blast powder), it is effective to combine the acid cleaning of cathode. After acid cleaning of anode or acid cleaning of cathode, the acid residue on the surface is flushed by water and cleaned. In the present invention, it is necessary to set up the time for cleaning within 20 seconds. When the time for cleaning is longer than 20 seconds, the length of treating zone becomes too long and the space reduction, which is one of the object of the present invention, can not be realized.

In the present invention, after cleaning process of metal wire rod, the metal wire rod is contacted with aqueous lubricious film forming treatment solution. Before the contact with this aqueous lubricious film forming treatment solution, it is desirable to preheat the metal wire rod. By this preheating the time for drying can be shortened, because the drying of the aqueous lubricious film forming treatment solution can be accelerated by preheating. The effect of shortening of drying time becomes more remarkable, because the space for this treating equipment can be reduced when the treating speed becomes higher,

As the specific method for this preheating, high-frequency heating, hot air heating, hot water bath heating, steam heating, direct heating or superheated steam heating can be applied. This preheating is carried out so as the temperature of metal wire rod to be from 70°C to 150°C. When the temperature of the metal wire rod is under 70°C, it is difficult to accelerate the drying after contacted with the lubricious film forming treatment solution, further, when the temperature of metal wire rod exceeds 150°C, since vapor generates by contacting the lubricious film forming treatment solution with the metal wire rod, normal lubricious film can not be formed. The effect of shortening of drying time by said preheating becomes more remarkable, because the space for this treating equipment can be reduced when the treating speed becomes higher.

The aqueous lubricious film forming treating solution used in the present invention contains inorganic salt and a slipping gent as main components. The lubricious film, which is the object of the present invention, is required to be good at follow-up ability during the plastic processing, to have hardness and strength against burning and sticking with a mold, to have good slipping ability and to reduce frictional coefficient. And for realization of these subjects, it is very important to use inorganic salt and a slipping agent in combination. As the inorganic salt, at least one selected from the group consisting of phosphate, sulfate, borate, molybdate and tungstate can be desirably used. Specifically, for example, zinc phosphate, calcium phosphate, sodium sulfate, potassium sulfate, potassium silicate, sodium borate (sodium tetra borate), potassium borate (potassium tetra borate), ammonium borate (ammonium tetra borate) ammonium molybdate, sodium molybdate and sodium tungstate can be mentioned. These compounds ca be used alone or can be used in combination.

As the slipping agent, metal soap, wax, fluororesin such as polytetrafluoroethylene, molybdenum disulfate and graphite are desirably used. These compounds can be used together with. Specifically, as the metal soap, compound obtained by reacting saturated fatty acid of carbon number from 12 to 26 with at least one metal selected from the group consisting of zinc, calcium, barium, aluminum, magnesium and lithium, for example, calcium stearate, zinc stearate, barium stearate, magnesium stearate and lithium stearate, can be mentioned. As the wax, micro crystalline wax, polyethylene wax, polypropylene wax and camauba wax can be mentioned. While, regarding PTFE, molybdenum disulfide and graphite, there is no limitation in average particle size or molecule weight.

Regarding the mixing ratio of slipping agent and inorganic salt in the lubricious film forming treatment solution, it is necessary to limit the ratio of slipping agent/inorganic salt within from 0.1 to 4.0 by solid weight ratio. When this solid weight ratio is less than 0.1, the slipping property is inferior and sufficient lubricity can not be obtained. And when the solid weight ratio excesses 4.0, since indent scratches are easily generated, it is not desirable. Desirable solid weight ratio is from 0.2 to 1.5. The slipping agent and the inorganic salt are used as the aqueous treating solution which are dissolved or dispersed in water. The public known surfactant or stabilizer can be used. As the surfactant, nonionic surfactant, anionic surfactant or cationic surfactant can be used.

As the nonionic surfactant, for example, polyoxyethylenealkylester prepared by polyoxyethylenealkylether, polyoxyalkylene(ethylene and/or propylene)alkylphenylether or polyethyleneglycol (or ethylene oxide) and high fatty acid (e.g. carbon number 12-18) or polyoxyethylenesorbitane alkyl ester prepared by sorbitane, polyethyleneglycol and high fatty acid (e.g. carbon number 12-18) can be mentioned, however, not intending to be limited to them. As the anionic surfactant, for example, fatty acid salt, sulfate salt, sulfonate salt, phosphate salt or dithio phosphate salt can be mentioned, however, not intending to be limited to them. As the amphoteric surfactant, for example, amino acid type and betaine type carboxylate salt, sulfate salt, sulfonate salt or phosphate salt can be mentioned, however, not intending to be limited to them. As the cationic surfactant, for example, fatty acid amine salt or tertiary ammonium salt can be mentioned, however, not intending to be limited to them. These surfactants can be used alone or can be used in combination.

Additionally, it is possible to add public known viscosity improving agent aiming to support the formation of film, if necessary, For example, in the case when it is necessary to improve smoothness and to control the unevenness of film, addition of a viscosity improving agent is effective. Further, it is possible to add polymer compound as the binder component, for the purpose to improve the adhesion of the film. The blending amount or a kind of these components are not specifically limited. For example, inorganic substance such as smectite clay mineral (montmolillonite, sauconite, beidelite or hectorite) and organic substance such as urethanes (polymer of polyol and polyisocyanate), poly carboxylic acid salts (polymer of acrylic acid, methacrylic acid, maleic acid or itaconic acid), polyolefins (polyvinyl alcohol), polyethers (polyethylene glycol, or polypropylene gricol) and polysaccharide (methyl cellulose, methyl starch or methyl guagum) can be mentioned.

In the present invention, it is necessary to limit the contact time with this aqueous lubricious film forming treatment solution within 5 seconds. When the contact time is over than 5 seconds, the treating zone becomes too long and the space reduction, which is one of the objects of the present invention can not be accomplished. The adhering amount of the lubricious film of the present invention is necessary to be limited within the limit of 0.5 to 20 g/m². When the adhering amount is smaller than 0.5 g/m², the sufficient lubricity can not be displayed. Further, when the adhering amount exceeds 20 g/m², the film becomes too thicker and causes indent scratches or surplus refuse, and is not desirable. The adhering amount of the lubricious film is adjusted to the desired adhering amount by regulating the coating amount and the concentration of the lubricant. The adhering amount can be easily calculated as follows. That is, cut the treated wire rod to the specific length and weight, then peel of the film. Calculate the adhering amount from the weight difference and the surface area (calculated from the cut length).

In the present invention, the wire rod to which lubricious film forming treating solution is adhered is dried, thus the lubricious film is formed on the surface of the wire rod. The method for drying is not specifically restricted, however, the drying by hot air is simple and desirable. Further, after treatment, the treated wore rod can be wound up, or can be continuously processed by drawing process, skinpath process or header process. Furthermore, the linear velocity of the metal wire rod at the continuous treatment is desirable to be in the limit from 10 to 150 m/min. When the linear velocity is less than 10 m/minute, since the sufficient productivity can not be obtained, not meets to the industrial use. In the meanwhile, when the linear velocity exceeds 150 m/min, since the uniformity after coating treatment of the lubricious film becomes deteriorated, it is not desirable.

The present invention will be illustrated more specifically according to the Examples and the Comparative Examples.

### (1) The material (wire rod) used in Examples and Comparative Examples.

① Steel material for drawing
   S45C spherical annealed steel: 3 mm diameter, 20 m length
② Stainless steel material for drawing
   SUS430: 3 mm diameter, 20 m length
③ Titanium material for drawing
   β alloy Ti-15V-3Cr-3Sn-3Al: 3 mm diameter, 20 m length
④Steel material for bolt
   SCM435: 9 mm diameter, 300 m length

### (2) Components of the lubricious film forming solution used in Examples and Comparative Examples

Treating solution 1
   Inorganic salt: sodium tetra borate
   Slipping agent: sodium stearate
   Ratio of slipping agent/inorganic salt: 1.0
   Concentration of solid: 10%
Treating solution 2
   Inorganic salt: zinc phosphate + sodium tetra borate (wt. ratio: 1:2)
   Slipping agent: sodium stearate + calcium stearate (wt ratio: 1:1)
   Ratio of slipping agent/inorganic salt: 0.5
   Concentration of solid: 5%
Treating solution 3
   Inorganic salt: potassium tetra borate
   Slipping agent: micro crystalline wax
   Ratio of slipping agent/inorganic salt: 2.0
   Concentration of solid: 10%
Treating solution 4
   Inorganic salt: potassium sulfate + potassium tetra borate (wt. ratio: 1:2)
   Slipping agent: PTFE
   Ratio of slipping agent/inorganic salt: 0.3
   Concentration of solid: 15%
Treating solution 5
   Inorganic salt: potassium silicate
   Slipping agent: calcium stearate + polyethylene wax (wt. ratio: 1:2)
   Ratio of slipping agent/inorganic salt: 1.5
   Concentration of solid: 15%
Treating solution 6
   Inorganic salt: sodium tetra borate
   Slipping agent: no
   Ratio of slipping agent/inorganic salt: 0
   Concentration of solid: 10%
Treating solution 7
   Inorganic salt: no
   Supping agent: polyethylene wax
   Ratio of slipping agent/inorganic salt: -
   Concentration of solid: 10%
Treating solution 8
   Inorganic salt: sodium tetra borate
   Slipping agent: sodium stearate
   Ratio of slipping agent/inorganic salt: 1.0
   Concentration of solid: 0.5%

### Examples 1-3

Above mentioned materials (wire rod) were processed by following processes ① to ⑤ in order. The linear velocity for treatment was 40 m/min.
① Acid cleaning of anode: 20% sulfuric acid, temperature 60°C, time 1 second, current density 30A/dm².
② Acid cleaning of cathode: 20% sulfuric acid, temperature 60°C, time 4 seconds, current density 40A/dm³.
③ Washing by water: By city water, 60°C, dipping time 5 minutes.
④ Surface treatment: Treating solution 1 (Example 1), 2 (Example 2) or 3 (Example 3) were used. 60°C, dipping time 2 seconds.
⑤ Drying: Hot air of 140°C was blown, 15 seconds.

### Examples 4-5

Above mentioned materials (wire rod) were processed by following processes ① to ③ in order. The linear velocity for treatment was 40 m/min.
① Shot blast: Shot ball ( ⌀ 0.5mm), time 10 minutes, pressure 5kgf/cm².
② Surface treatment: Treating solution 4 (Example 4) or 5 (Example 5) were used. 60°C, dipping time 2 seconds.
③ Drying: Hot air of 140°C was blown, 15 seconds.

### Examples 6-8

Above mentioned materials (wire rod) were processed by following processes ① to ⑤ in order. The linear velocity for treatment was 100 m/min.
① Bending: 90° bending (4 steps)
② Acid cleaning of cathode: 20% sulfuric acid, temperature 60°C, time 2 seconds, current density 100A/dm².
③ Washing by water: By city water, 60°C, dipping time 3 minutes.
④ Surface treatment: Treating solution 1 (Example 6), 2 (Example 7) or 3 (Example 8) were used. 60°C, dipping time 1 second.
⑤ Drying: Induction heating (2 seconds), reached temperature 120°C.

### Examples 9-10

Above mentioned materials (wire rod) were processed by following processes ① to ④ in order. The linear velocity for treatment was 40 m/min.
① Shot blast: Shot ball (⌀ 0.5mm), time 10 minutes, pressure 5kgf/cm².
② Preliminary heating: Hot water bath (temperature 90°C), dipping 3 seconds.
③ Surface treatment: Treating solution 4 (Example 9) or 5 (Example 10) were used. 60°C, dipping time 1 second.
④ Drying: Hot air of 140°C was blown, 3 seconds.

### Examples 11-12

Above mentioned materials (wire rod) were processed by following processes ① to ④ in order. The linear velocity for treatment was 100 m/min.
① Shot blast: Shot ball (⌀0.5mm), time 5 minutes, pressure 7kgf/cm³.
② Preliminary heating: Induction heating (1 second), reached temperature 80°C.
③ Surface treatment: Treating solution 4 (Example 11) or 5 (Example 12) were used. 60°C, dipping time 1 second.
④ Drying: Hot air of 200°C was blown, 2 seconds.

### Comparative Examples 1, 2

Above mentioned materials (wire rod) were processed by following processes
① to ⑤ in order. The linear velocity for treatment was 40 m/min.

① Acid cleaning of anode: 20% sulfuric acid, temperature 80°C, time 1 second, current density 30A/dm².
② Acid cleaning of cathode: 20% sulfuric acid, temperature 60°C, time 4 seconds, current density 40A/dm².
③ Washing by water: By city water, 60°C, dipping time 5 minutes.
④ Surface treatment: Treating solution 6 (Comparative Example 1) or 7 (Comparative Example 2) were used. 60°C, dipping time 2 seconds.
⑤ Drying: Hot air of 140°C was blown, 15 seconds.

### Comparative Example 3

Above mentioned materials (wire rod) were processed by following processes ① to ② in order. The linear velocity for treatment was 40 m/min.
① Surface treatment: Treating solution 1 was used. 60°C, dipping time 3 seconds.
② Drying: Hot air of 140°C was blown, 15 seconds.

### Comparative Example 4

Above mentioned materials (wire rod) were processed by following processes ① to ③ in order. The linear velocity for treatment was 200 m/min.
① Shot blast: Shot ball (⌀0.5mm), time 10 minutes, pressure 5 kgf/cm².
② Surface treatment: Treating solution 8 was used. 60°C, dipping time 3 seconds.
③ Hot air of 140°C was blown, 15 seconds.

### Comparative Example 5

Above mentioned materials (steel ①, ④) were processed by following processes ① to ⑧ in order.
① Alkali Degreasing: Degreasing agent on the market (T.M. Fine Cleaner 4360: Product of Japan Parkerizing Co., Ltd.) concentration 20g/L, temperature 60°C, dipping time 10 minutes.
② Washing by water: City water, ordinary temperature, dipping time 10 minutes.
③ Acid cleaning: 17% hydrochloric acid, temperature 30°C, dipping time 10 minutes.
④ Washing by water: City water, ordinary temperature, dipping time 5 minutes.
⑤ Chemical conversion treatment: Zinc phosphate chemical conversion treating agent on the market (T.M. PALBOND 3670X: Product of Japan Parkerizing Co., Ltd.) concentration 90 g/L, temperature 80°C, dipping time 10 minutes.
⑥ Washing by water: City water, ordinary temperature, dipping time 5 minutes.
⑦ Treatment by soap: Reactive soap lubricant agent on the market (T.M. PALUVE 285: Product of Japan Parkerizing Co., Ltd.) concentration 70 g/L, temperature 80°C, dipping time 5 minutes.
⑧ Drying: Hot air of 80°C blow, 20 minutes.

### Comparative Example 6

Above mentioned material (stainless steel ②) was processed by following processes ① to ⑧ in order.
① Alkali Degreasing: Degreasing agent on the market (T.M. Fine Cleaner 4360: Product of Japan Parkerizing Co., Ltd.) concentration 20g/L, temperature 60°C, dipping time 10 minutes.
② Washing by water: City water, ordinary temperature, dipping time 10 minutes.
③ Acid cleaning, Nitric acid - hydrofluoric acid (10% nitric acid - 5% hydrofluoric acid), ordinary temperature, dipping time 10 minutes.
④ Washing by water: City water, ordinary temperature, dipping time 5 minutes.
⑤ Chemical conversion treatment: Oxalate chemical conversion treating agent on the market (T.M. FELBOND A: Product of Japan Parkerizing Co., Ltd.) concentration of 1 agent is 30g/L and concentration of 2 agent is 15g/L, temperature 95°C, dipping time 5 minutes.
⑥ Washing by water: City water, ordinary temperature, dipping time 5 minutes.
⑦ Treatment by soap: Reactive soap lubricant agent on the market (T.M. PALUVE 235: Product of Japan Parkerizing Co., Ltd.) concentration 70 g/L, temperature 80°C, dipping time 5 minutes.
⑧ Drying: Hot air of 80°C blow, 20 minutes.

### Comparative Example 7

Above mentioned material (steel ③) was processed by following processes ① to ⑧ in order.
① Alkali Degreasing: Degreasing agent on the market (T.M. Fine Cleaner 815: Product of Japan Parkerizing Co., Ltd.) concentration 15 g/L, temperature 60°C, dipping time 10 minutes.
② Washing by water: City water, ordinary temperature, dipping time 10 minutes.
③ Acid cleaning: Nitric acid - hydrofluoxic acid (10% nitric acid - 5% hydrofluoric acid), ordinary temperature, dipping time 10 minutes.
④ Washing by water: City water, ordinary temperature, dipping time 5 minutes.
⑤ Chemical conversion treatment: Chemical conversion treating agent on the market (T.M. PALMET 3855: Product of Japan Parkerizing Co., Ltd.) concentration 25g/L, temperature 60°C, dipping time 10 minutes.
⑥ Washing by water: City water, ordinary temperature, dipping time 5 minutes.
⑦ Treatment by soap: Molybdenum lubricant on the market (T.M. PALUVE 4649C: Product of Japan Parkerizing Co., Ltd.) concentration 800 g/L, temperature 80°C, dipping time 3 minutes.
⑧ Drying: Hot air of 80°C blow, 20 minutes.

The metal wire rods obtained in above Examples 1-12, Comparative Examples 1-7 are respectively evaluated as follows. And the results are summarized in Table 1.

### <Evaluation>

### · Drawability

Three steps processing is carried out on wire rod. Evaluated by imperfection after third step drawing and by the load (Kgf) at the third drawing. No imperfection and low drawing load is highly evaluated.
1^{st} step: ⌀3.00mm→⌀2.76mm
2^{nd} step: ⌀2.76mm→⌀2.40mm
3^{rd} step: ⌀2,40mm→⌀2.17mm

### · Header processability

Skinpath process is carried out on wire rod for a bolt processing (to ⌀ 8.3), then 200 pieces of bolt shown in Table 1 are produced continuously by a conventional header machine using former oil. Whether there is an imperfection on the top portion of the bolt or not is inspected by eyes of the inspector, and the numbers of pieces which have an imperfection and the degree of the imperfection is checked.

### · Numbers of process

Evaluation is performed by considering the numbers of process and the space of the equipment. Smaller numbers of process and narrower space are desirable.

### · Environmental protection

Evaluated by whether there is sludge to be wasted or not. No sludge to be wasted is desirable.

As clearly understood from Table 1, the Examples 1 to 12, which depend on the method for preparation of the metal wire rod for plastic processing of the present invention display excellent lubricity, the occupancy space for equipment is small and superior in environmental protection. In the cases of Examples 9 and 10, since the time necessary for the treatment in whole processes can be shortened by carrying out the previous heating, the occupancy space of the treating equipment can be reduced.
Further, in the cases of Examples 11 and 12, although the treating speed is 2.5 times to that of Examples 4 and 5, the occupancy space of the treating equipment is only 1.5 times to that of Examples 4 and 5. This is basically the effect of shortening of treating time caused by the previous heating process.

In the cases of Comparative Examples 1 and 2, whose lubricant/inorganic salt ratio is out of the limit of the present invention, are inferior in lubricity and cause partial burning and sticking with the mold at the drawing process, further it is difficult to carry out the header process. And, in the case of Comparative Example 3, which omit the cleaning treatment, the lubricity is not sufficient so as to carry out the processing is impossible. Still further, in the case of Comparative Example, whose adhering amount is out of the limit of the present invention, the lubricity is not sufficient and is impossible to carry out the processing. Regarding the cases of Comparative Examples 4 to 7, which are the conventional art, although the lubricity is good, there are problems from the view point of the occupancy space and the environmental protection.

### INDUSTRIAL APPRICABILITY

By the method for preparation of metal wire rod for plastic processing of the present invention, it is possible to generate the film having high lubricity by simple treatment and by short time. Further, from the view point of the earth environment, saving energy and saving space, the industrial applicability is extremely large.

## Claims

1. A method for preparation of the metal wire rod for plastic processing comprising, carrying out cleaning treatment by at least one kind of cleaning treatment method selected from the group consisting of shot blast, sand blast, bending and acid cleaning of cathode and anode on the surface of metal wire rod of 0.3-50 mm diameter for 20 seconds or less, contacting with aqueous lubricious film formation treating solution which contains at least one kind of inorganic salt selected from the group consisting of phosphate, sulfate, borate, silicate, molybdate or tungstate and at least one kind of slipping agent selected from the group consisting of metal soap, wax, polytetrafluoroethylene, molybdenum disulfate and graphite, wherein the weight ratio of solid of said slipping agent/inorganic salt is within the limit from 0.1 to 4.0, for 5 seconds or less, drying immediately and forming lubricious film of adhesion amount from 0.5 to 20 g/m² on the surface of the wire rod by continuous inline system.

2. A method for preparation of the metal wire rod for plastic processing comprising, carrying out cleaning treatment by at least one kind of cleaning treatment method selected from the group consisting of shot blast, sand blast, bending and acid cleaning of cathode and anode on the surface of metal wire rod of 0.3-50 mm diameter for 20 seconds or less, carrying out previous heat treatment, then contacting with aqueous lubricious film formation treating solution which contains at least one kind of inorganic salt selected from the group consisting of phosphate, sulfate. borate, silicate, molybdate or tungstate and at least one kind of slipping agent selected from the group consisting of metal soap, wax, polytetrafluoroethylene, molybdenum disulfate and graphite, wherein the weight ratio of solid of said slipping agent/inorganic salt is within the limit from 0.1 to 4.0, for 6 seconds or less, drying immediately and forming lubricious film of adhesion amount from 0.5 to 20 g/m² on the surface of the wire rod by continuous inline system.

3. The method for preparation of the metal wire rod for plastic processing of claim 1 or claim 2, wherein the metal wire rod is selected from the group consisting of iron, steel stainless steel, aluminum, aluminum alloy, magnesium, magnesium alloy, titanium, titanium alloy, copper or copper alloy.

4. The method for preparation of the metal wire rod for plastic processing according to anyone of claims 1 to 3, wherein the linear velocity of metal wire rod at the continuous treatment is from 10 to 150 m/minute.
